

## 1

## 3,726,671

## SEALING ALLOY

George A. Majesko, Glen Ridge, N.J., assignor to  
 Wilbur B. Driver Company  
 No Drawing. Filed Jan. 15, 1971, Ser. No. 106,897  
 Int. Cl. C22c 39/10

U.S. CL. 75—134 F

3 Claims

## ABSTRACT OF THE DISCLOSURE

A glass sealing alloy comprising, as expressed in percent by weight, the following major constituents:

|          | Percent   |
|----------|-----------|
| Nickel   | 5.5—20.0  |
| Cobalt   | 42.5—57.0 |
| Chromium | 5.0—6.5   |
| Iron     | Balance   |

the sum of the nickel and cobalt constituents falling within the range 62.0%—63.0%.

## BACKGROUND OF THE INVENTION

In order to provide a satisfactory hermetic seal between the glass envelope of an electron device and electrical leads or pins, a sealing alloy known as 52 alloys is conventionally used. This is an essentially binary alloy containing 52% of weight of nickel, balance iron. However, seals of this type can exhibit a tendency to leak due to incomplete or insufficient adherence of the metal oxide whereby the hermeticity is destroyed. The exposed surfaces of this sealing alloy have poor corrosion resistance in most environments.

I have discovered that a quaternary alloy having nickel, iron, cobalt and chromium components can be used to overcome this difficulty. More particularly, this new alloy is characterized by the ability to form tight, adherent hermetic bonds in glass to metal seals, and also exhibits the same thermal expansion properties as 52 alloy. Moreover, my alloy exhibits enhanced corrosion resistance in most environments. As a result, my alloy can be substituted for 52 alloy in sealing applications with the advantages indicated.

## SUMMARY OF THE INVENTION

In accordance with the principles of my invention, my alloy comprises the following major constituents as expressed in percent by weight:

|        | Percent   |
|--------|-----------|
| Nickel | 5.5—20.0  |
| Cobalt | 42.5—57.0 |

the sum of the nickel and cobalt constituents falling within the range 62.0%—63.0%;

|          |         |
|----------|---------|
| Chromium | 5.0—6.5 |
| Iron     | Balance |

The alloy contains up to 1% of certain minor constituents including:

|           |       |
|-----------|-------|
| Manganese | 0—0.5 |
| Silicon   | 0—0.4 |

This alloy forms a single phase, solid solution and is characterized by a thermal coefficient of expansion falling within the range, expressed in parts per million per degree centigrade (p.p.m./° C.), of 8 p.p.m./° C. to 11 p.p.m./° C. over the temperature range of about 30° C. to 550° C. As a result, my alloy can be used in forming glass to metal hermetic seals with glasses having essentially the same thermal coefficients of expansion over the same temperature range.

## 2

## DETAILED DESCRIPTION OF PREFERRED EMBODIMENTS

One typical alloy composition in accordance with my invention is as follows:

|            | Percent |
|------------|---------|
| Nickel     | 14.0    |
| Cobalt     | 48.5    |
| Chromium   | 6.0     |
| 10 Silicon | 0.1     |
| Manganese  | 0.35    |
| Iron       | Balance |

The thermal coefficient of expansion of this composition, from 25° C. to 450° C., was found to be 9.79 p.p.m./° C. The thermal coefficient of expansion of 52 alloy is essentially the same. However, my alloy can be used to provide enhanced adherence and hermetic bonding as previously indicated. My alloy forms a stable, single phase, solid solution. Providing that the major constituents of my alloy are held within the ranges recited above, the expansion coefficient will be held within the range 8 p.p.m./° C. to 11 p.p.m./° C., and the alloy will not undergo any allotropic transformations. Moreover my alloy is much less susceptible to corrosion attack.

As a specific example, for 15 minutes in 20% nitric acid at 180° F., using samples having equivalent surface areas, the 52 alloy showed 17.3% weight loss as compared to only .02% weight loss for my alloy. Advantages can also be shown in other corrosive environments.

The minor constituents should be held within the ranges indicated below:

|            | Percent |
|------------|---------|
| Manganese  | 0—0.5   |
| 35 Silicon | 0—0.4   |

Chromium is added to enhance the adherence of the oxide formed in making glass to metal seals. Below 5% chromium, there is little enhancement. Additions of chromium in excess of 6.5% produces no further enhancement. In addition, these chromium additions have a passivating effect in comparison to 52 alloy whereby my alloy is more corrosion resistant.

Unless the sum of the nickel and cobalt constituents of my alloy is held within the range 62.0%—63.0%, the curie temperature and related inflection temperature will not be maintained at the same values as in the 52 alloy, and the resultant thermal coefficient of expansion will fall outside the desired range.

When the sum of nickel and cobalt is held between 62% and 63%, the lower limit of Ni is 5.5%. When the nickel content falls below this value, the alloy is likely to be a two phase structure as opposed to a single phase structure. The expansion behavior of a two phase structure can be unstable and unpredictable.

The upper limit of the nickel content is 20%. When nickel is substituted for cobalt and the sum of these two constituents is held within the range 62.0%—63.0%, nickel additions in excess of 20% produce expansion coefficient which are too high.

My alloy can be produced by the same procedures as required for 52 alloy. No special precautions are necessary, but the alloy should be clean and relatively defect free.

While I have described my invention with particular reference to preferred embodiments, my protection is limited only by the terms of the claims which follow.

What is claimed is:

1. An alloy, as expressed in percent by weight, consisting essentially of:

|        | Percent   |
|--------|-----------|
| Nickel | 5.5—20.0  |
| Cobalt | 42.5—57.0 |

## 3

the sum of the nickel and cobalt falling within the range 62.0%–63.0%.

|         | Percent |
|---------|---------|
| Cromium | 5.0–6.5 |
| Silicon | Balance |

2. An alloy as set forth in claim 1 further including:

|           | Percent |
|-----------|---------|
| Manganese | 0–0.5   |
| Silicon   | 0–0.4   |

3. An alloy as set forth in claim 2 containing:

|            | Percent |
|------------|---------|
| Nickel     | 14      |
| Cobalt     | 48.5    |
| Chromium   | 6.0     |
| Silicon    | 0.1     |
| Managanese | 0.35    |

## 4

## References Cited

## UNITED STATES PATENTS

|             |         |           |           |
|-------------|---------|-----------|-----------|
| 1,841,097   | 1/1932  | Elmen     | 75—123 K  |
| 2,044,165   | 6/1936  | Halliwell | 75—123K X |
| 5 2,065,404 | 12/1936 | Scott     | 75—170 X  |

## FOREIGN PATENTS

|         |         |               |          |
|---------|---------|---------------|----------|
| 357,665 | 10/1931 | Great Britain | 75—123 K |
|---------|---------|---------------|----------|

L. DEWAYNE RUTLEDGE, Primary Examiner

J. E. LEGRU, Assistant Examiner

U.S. Cl. X.R.

15 75—122, 171